

# UNITED STATES PATENT OFFICE.

EDWARD GOODRICH ACHESON, OF NEW YORK, N. Y.

## SOAP COMPOSITION AND PROCESS OF MAKING SAME.

1,419,952.

Specification of Letters Patent. Patented June 20, 1922.

No Drawing.

Application filed October 5, 1920. Serial No. 414,915.

To all whom it may concern:

Be it known that I, EDWARD GOODRICH ACHESON, a citizen of the United States, residing at New York, in the county of New York and State of New York, have invented certain new and useful Improvements in Soap Compositions and Processes of Making Same, of which the following is a specification.

10 This invention is a novel soap composition comprising in addition to the fatty acid salts of the alkali metals, constituting the body of the soap or soap-stock, a certain admixture of clay particles which have undergone deflocculation in accordance with the processes disclosed in my prior United States patents and now well understood by those skilled in this art. The invention comprises also the process of preparing the 20 above composition. In the preferred embodiment of the present invention the clay particles which have undergone deflocculation, and have been thereby transformed to the permanently suspensible or colloidal 25 state, are "re-flocculated" or converted into extremely minute and fragile but nevertheless filterable aggregates or flocks before being incorporated with the soap stock.

For use in accordance with the present 30 invention I prefer to employ the novel clay product described and claimed in my co-pending application Serial No. 414,914, filed October 5, 1920. A product of this kind may be prepared as disclosed in the said application or as follows:

Fine clay preliminarily freed from sand or grit, is subjected to a process of attrition in a moist state and in presence of a deflocculating agent, the latter preferably comprising such products as may be extracted from roasted starchy materials by the action of aqueous ammoniacal solutions, methyl-amine solutions or the like. This treatment of the clay may be performed in accordance with my prior United States patents numbered 1,223,350; 1,253,556; 1,345,305 and 1,345,360.

The entire product from the deflocculating mill, referred to in practice as the "mill-paste," and comprising a mixture of non-deflocculated or partially deflocculated with fully deflocculated particles, is transferred to an agitator in which it is mixed with water and thoroughly stirred, and thence discharged into a classifying device, preferably a Dorr thickener.

The finer and lighter effluent from the thickener comprises the fully deflocculated or permanently suspensible (colloidal) particles resulting from the deflocculating operation, and also those particles which sufficiently approximate this condition to remain suspended in the water under the classifying conditions. This effluent is run into a settling tank, preferably of wood, and receives a small addition of a flocculating agent (electrolyte) such for example as a mineral acid, alum, sodium chlorid or the like.

The whole of the solid material, including that which has undergone deflocculation, is thereby precipitated, and may be collected upon a vacuum filter, and if desired further dried in an oven or other appropriate drying apparatus. This material is that which I employ as a component of my novel soap compositions. It is readily distinguishable from the components separated from clay, by ordinary method of levigation and washing, being not only more minutely and evenly subdivided, but also, it is believed, more readily subdivisible into still finer particles, this latter characteristic being attributed to the very delicate and extremely frangible nature of the aggregates resulting from the re-flocculation step. Microscopically, these appear to be loosely coherent masses composed of extremely minute particles.

In my preferred procedure as described above, the re-flocculation takes place in presence of residual non-deflocculated or only partially deflocculated material, this resulting in a very intimate admixture of fine particles, a portion only of which have undergone full deflocculation. It is however within the scope of my invention to effect a substantially complete separation between the fully deflocculated and non-deflocculated particles, as for example by permitting the latter to subside from a suspension of the former, drawing off the suspension and then reprecipitating the deflocculated suspension by the addition of an electrolyte as already described. For most purposes however such a refinement of the process is unnecessary.

It is known that ordinary clay, added to soap stock in proportion to constitute up to 30-40% or even more of the whole, tends to improve the detergent and cleansing qualities of the soap. I have found however that certain added effects are produced when the clay, or a portion of it, has passed

through the deflocculated state as a treatment preparatory to its incorporation in the soap stock. Notable among these effects are the tendency to the formation of smooth and unctuous films which persist until removed by rinsing; and the formation of relatively strong and permanent lathers. Without limiting the invention by any theoretical considerations, I now attribute this latter characteristic to the fact that my clay product, prepared as described herein, consists or contains a large proportion of particles of such minute size that they are capable of being actually enclosed within or floated by the liquid films which constitute the bubble walls. It is well known that the forces governing adhesion between solids and liquids, in cases where the solids are wetted by the liquids, are of a decidedly higher magnitude than those governing the cohesion of liquids; hence when readily wetted particles are introduced into a bubble-forming liquid, and are of an order of magnitude to be enclosed within and carried by the walls of the bubbles, the resultant effect is to strengthen the bubble to the extent that the adhesive forces are superposed upon or

added to the cohesive forces. The clay particles in the lather prepared from the herein-described soap-compositions are believed to be largely of this order of magnitude, but as already stated my invention is not restricted to such considerations of theory.

I claim:—

1. A soap-composition, comprising soap- stock and a clay addition, the latter comprising particles reprecipitated from the deflocculated state. 35

2. Process of making a soap-composition, comprising subjecting clay to a deflocculating operation, whereby a portion of the same is transformed to the colloidal state; then reflocculating the colloidal clay, and incorporating the product with soap stock. 40

3. Process of making a soap-composition, comprising subjecting clay to a deflocculating operation, whereby a portion of the same is transformed to the colloidal state; then reflocculating the colloidal clay in presence of the residual fine material, and incorporating the product with soap-stock. 45

In testimony whereof, I affix my signature.

EDWARD GOODRICH ACHESON.